

Jan. 10, 1950

J. MAGNIN

2,493,768

METHOD OF LEAD COATING

Filed June 21, 1944.

3 Sheets-Sheet 1

Fig. 1.



Fig. 2.



Inventor  
Jacques Magnin

by Steel Jackson and Son  
Attorneys

Witnesses:  
Louis Wallin  
Walter Chion.

Jan. 10, 1950

J. MAGNIN

**2,493,768**

## METHOD OF LEAD COATING

Filed June 21, 1944

3 Sheets-Sheet 2



Witnesses:  
Doris Wallin  
Walter Chenu.

Inventor  
Jacques Magnin  
by ~~Att~~ - Stark Jackson and Son  
Attorneys.

Jan. 10, 1950

J. MAGNIN

2,493,768

#### METHOD OF LEAD COATING

Filed June 21, 1944

3 Sheets-Sheet 3



Witnesses:  
Doris Wallin  
Walter Chisum

Inventor  
Jacques Magnin  
by ~~of~~ Field Palmer and Son  
Attorneys.

## UNITED STATES PATENT OFFICE

2,493,768

## METHOD OF LEAD COATING

Jacques Magnin, Chestnut Hill, Pa., assignor to  
Horace C. Knerr

Application June 21, 1944, Serial No. 541,348

6 Claims. (Cl. 117—52)

1 My invention relates to coating metal parts with lead as a lubricant to facilitate successive cold working operations changing the shape of the metal without necessity for intermediate annealings and/or picklings. Commercially pure lead is ordinarily used.

The main purpose of the invention is to produce a surface which is coated with lead and in which the lead adheres even after numerous cold passes.

A further purpose is to perform the lead coatings of metals in a single operation.

A further purpose is to avoid the necessity for preliminary wet bath treatment before actual lead coating and to use a dry bath treatment only.

A further purpose is to apply acetates, borates, chlorides or sulphates of antimony, bismuth, cadmium or tin floating upon the surface of a molten bath of lead, as a means of preparing the surface of iron and of metal alloys generally for a coating of lead for lubricating purposes, and to use various salts of iron for the same purpose.

A further purpose is to apply stannous chloride, stannic chloride, cadmium chloride or antimony chloride as fluxes having affinity both for iron when it is being lead coated and for the lead coating and thus to facilitate the coating operation and produce more permanent and better results than could otherwise be attained.

A further purpose is to coat with lead from a molten bath of lead, and for purposes of lubrication with the aid of a molten flux floating on the surface of the lead and containing chlorides, borates and sulphates of antimony, bismuth, cadmium or tin, heating parts to be coated within the molten flux and passing them through it into the molten lead, withdrawing from an uncoated surface of the lead or through the flux as may be preferred.

A further purpose in lead coating for lubrication is to pass metal objects to be lead coated through a bath containing zinc chloride and stannic or stannous chloride, cadmium chloride or antimony chloride as an alloying flux, facilitating coating with lead upon steel, copper or brass, chrome-iron and nickel-chrome, for example, reducing the cost of the coating, the time and handling required and the space occupied by the operation.

A further purpose is to unite a lead coating to steel, iron, copper, brass, nickel-chrome, chrome-iron alloys and non-ferrous alloys generally at a lower cost and in shorter time than previously have been available.

2 A further purpose is to eliminate the use of mercury compounds in dipping operations for coating metals with lead.

3 A further purpose is to eliminate hydrous baths other than such as pickling in preparation for ultimate dry bath treatment coating lead upon various metals.

4 A further purpose is substantially to eliminate the use of ammonium compounds in a bath for dry treatment of metals to coat their surfaces with lead, using a trifling amount only to reduce the formation of oxides in the bath but permitting the use of much more where this is desired.

5 15 A further purpose is to dip the metals to be coated through the flux into the lead, to move the articles to be coated back and forth within the lead and flux and to advance the articles along a path from the position of flux covering to the position of ultimate withdrawal from the molten lead, passing them through the flux and bath repeatedly but finally withdrawing the articles which have been coated by the lead.

6 20 A further purpose is to pass the articles to be coated through the flux into the molten lead, to expose the articles to different parts of the lead bath while shifting them within it and finally to withdraw the articles through a lead surface free from flux coating.

7 25 A further purpose is to dip the articles by a mechanical dipping device such as a conveyor chain, to heat the device so that it will not chill the lead and to reciprocate the articles within the molten lead during their progress from a point at which they lie below the flux to a point at which they are withdrawn from the lead.

8 30 Further purposes will appear in the specification and in the claims.

9 35 Figure 1 is a sectional view of a treating pot showing a simple application of the preferred form of my invention.

10 40 Figure 2 is a sectional view showing a second form of my invention. Withdrawing the metal coated through the flux is objectionable according to the salts used in the flux. It reduces but does not destroy the lubricant function of the lead.

11 45 Figure 3 is a vertical section showing a form of the invention corresponding generally with Figure 1 but in which a mechanical dipping mechanism is used. The section is taken upon the line 3—3 of Figure 4.

12 50 Figure 4 is a fragmentary section of the structure of Figure 3 taken at right angles to that of Figure 3.

Figure 5 is a fragmentary section, largely a side elevation showing a ratchet mechanism seen in Figures 3 and 4.

In the drawings similar numerals indicate like parts.

This application is a continuation in part of my application for Process or method of lead coating, Serial No. 466,195, filed November 19, 1942, now abandoned. Related subject matter to the present application appears in my copending applications Serial No. 541,347, filed June 21, 1944, for Metallic lubrication; Serial No. 544,072, filed July 8, 1944, for Method and machine for lead coating; and Serial No. 544,073, filed July 8, 1944, now abandoned for Coating method.

In cold working of metals in order to bring them to the required shape and dimensions the metals usually have to be annealed, pickled and lubricated between each two succeeding cold working operations.

Ductile metals are hardened by cold work, and this is true notwithstanding differences in lubricants.

The degree of hardness produced in the initial stages of cold work is such that ordinary lubricants are inadequate to overcome the frictional resistance between the die, etc., and the metal. In such cases reannealing becomes a necessary operation. This ordinarily involves another pickling operation to remove the oxides produced by annealing.

Under this invention the coating of lead applied to the surface of the metal functions as a so much superior lubricant that frictional resistance is greatly reduced even after many successive cold passes.

With various metals initial cold work causes a great increase in hardness over that in the annealed condition but continued cold work does not correspondingly increase the hardness.

It has been found that coating certain metals such as iron, steel, copper, brass, chrome-iron, nickel-chrome alloys and non-ferrous alloys with lead generally acts as a lubricant in drawing tubing, or wire drawing, deep drawing, stamping, etc. by reason of which after the first annealing and pickling it is not necessary to repeat these operations after a considerable series of mechanical distortions during which the lead coating flows along with the metal but is not eliminated, with the result that even after as many as six or seven successive reductions or distortions the metal still shows a lubricating coating of lead.

A coating of lead upon the metal can be produced in various ways.

Another feature of importance is the fact that the lead adheres to the metal to such an extent that even when in the course of cold drawing operations the hardness of the metal becomes too great to carry on the cold work it is still possible to reanneal this metal (provided this is done in a controlled atmosphere) without destroying the lead coating. Therefore with the original lead coating from the start further cold drawing operations can still be performed with the original lead coating as lubricant. In retort annealing (or controlled atmosphere) the lead coating is not destroyed and does not form oxides and still retains its lubricating properties.

Pure lead can be electroplated upon the iron by electrolytic means but the adhesive qualities of this coating are not satisfactory. The deposit is pulverulent and crystalline and is rather easily removed. It is uneconomical as it requires an expensive plant and careful and constant super-

vision. It has the one advantage of unusual purity of the lead which is desirable in order that the full malleability may be attained; but the lead is not incorporated into the surface of the metal parts. Full retention of the lead requires a hold of the lead upon the metal similar to that secured by impregnation, by which the lead permeates the surface of the metal.

Another way in which attempt has been made to incorporate the lead to fasten the lead upon the surface of the metal is by alloying the lead with a small percent of tin or of antimony. Each of these alloying metals hardens the lead to such an extent as, in large measure, to defeat the lubricant effect of the lead upon the surface in subsequent mechanical operations performed upon the metal coated.

Coating of metals with lead alloys has been proposed in a series of patents in which the coating was planned for protective purposes but in which there seems to have been no thought of use as a lubricant and in which there is no such teaching. The character of coating planned was prohibitory for such a purpose inasmuch as the coating bath contained at least two percent of tin and two percent of antimony. One disclosure proposes ten percent of antimony and five percent of tin. In one of the patents a final passage of the coated material through a stannous chloride flux was contemplated for the express purpose of giving a thin coating of tin. Though the proportions of the bath were not given the material was constantly referred to as a solder. It evidently contained a large percentage of tin.

The purpose of the antimony and tin in these several disclosures was evidently to use the alloy with tin as a means of making the coating adhere to the surface of the metal to be coated.

Another method which has proved to be successful to a certain extent, after annealing and pickling, dips the metal to be coated in an aqueous solution (i. e. a "wet" bath) of bichloride of mercury saturated with zinc chloride as a preparatory step in the method, and subsequently passes the metal to be coated through a non-aqueous ("dry") molten flux floating on a molten lead bath. The flux contains zinc chloride and a considerable quantity of ammonium chloride.

The mercury process entails an additional operation and the cost of bichloride of mercury for the wet step of the process offsets a great part of the savings.

One of the difficulties with the bichloride of mercury treatment is that the slightest trace of grease before amalgamation prevents amalgamation, and if on the amalgamated surface (for instance from the handling of the metal with greasy gloves) prevents the lead from adhering. Furthermore the bichloride of mercury is a poison and is a dangerous chemical with which to deal.

I have discovered that excellent results can be attained by a dry dipping process without any preliminary wet process step such as, for example, a bichloride of mercury step. I use a salt derived from a metal which has affinity for (i. e. tends to alloy with) both the lead and the metal which is to be coated with the lead. I pickle in the usual way.

The salts preferably used are the chlorides, acetates, borates and sulphates.

Considering the price as well as the desirability, either molten stannic or molten stannous chloride floating on the molten lead gives good results, better than secured from others of the salts named. Either cadmium or antimony chloride

also gives good results. All three—use separately or permissibly together—give better results when used with zinc chloride than without it but will operate to lead coat the surface of the metal for lubrication purposes if used without zinc chloride. On the other hand zinc chloride will not lead coat the surface when used alone nor when used with ammonium chloride. The sulphates and borates of bismuth, antimony, cadmium, tin and iron have the same characteristics as the 10 chloride, will operate without zinc chloride—but better with it—and are improved by the presence of sodium chloride.

In my dipping operation I dip through a flux which may cover a part only of the surface of 15 the lead bath, so that the dipped metal may be withdrawn from a clear lead surface beyond a partition as in Figure 1; or the metal may be dipped into a completely flux-covered lead bath and withdrawn through the floating flux of the 20 same bath, as in Figure 2.

In Figure 1 the tank is shown at 5 with a content of molten lead 6 and a partition 7. The flux salts are shown at 8 on the entrance side of the partition and may comprise various salts in the 25 alternative, including stannous or stannic chloride or cadmium chloride or antimony chloride, or a borate or sulphate of cadmium, of bismuth, of antimony or of iron. Here again the operation is improved by the use of sodium chloride 30 and of zinc chloride. The clear surface of the bath beyond the partition is shown at 9.

In Figure 2 the pot is shown at 5' holding a molten lead 6 upon which a molten flux 8' floats, spreading over the entire lead bath. The form of Figure 2 has a disadvantage for lubricating purposes, made worse, of course, where the flux contains tin or any other metal which has a definite hardening effect, that where there is a definite layer of the flux left on the surface of the coating of lead, it reduces the lubricant quality of the coating of lead.

Because each of the metals, tin, cadmium and antimony, etc. has an affinity for (this may be but another way of stating "will form an alloy with") the metal to be coated and with lead, its salts form molten fluxes by which the surface of the metal can be covered with lead. This is true of metals generally, that they can be lead coated by dipping into a molten bath of commercially pure lead through a molten flux if the flux tends to alloy with the metal to be coated, and also with the lead.

The lead coated articles are then withdrawn from the lead bath and allowed to cool when they are ready for such operations as drawing, wire drawing, rolling or deep stamping without intermediate annealing, pickling and again lubricating.

Because other materials than lead, whether definitely hardening the surface of the lead or forming an alloy with lead of inferior lubricant quality or not, act as impurities to reduce the effectiveness of the lead as a lubricant, it is quite desirable to have pure lead. It is difficult, or at least expensive to get chemically pure lead but I have secured excellent results with a bath of what is known as commercially pure lead.

The principal benefit of my invention lies in the fact that the union of the lead with the outer part of the metal coated includes a permeation of the metal surface by the lead much like impregnation and possibly designated as impregnation. It may be a case of alloying with both metals.

The chlorides of the different metals used have been found to be the most suitable salts and at the same time the cheapest.

Some of the fluxes used successfully by me in lead coating have been as follows:

|                      | Parts                                                                            |
|----------------------|----------------------------------------------------------------------------------|
| Stannous chloride    | 1                                                                                |
| Zinc chloride        | 3                                                                                |
|                      | with a small addition from time to time of ammonium chloride to reduce oxidation |
|                      | Parts                                                                            |
| Cadmium chloride     | 1 to 2                                                                           |
| Zinc chloride        | 8 to 9                                                                           |
|                      | with a small addition from time to time of ammonium chloride                     |
|                      | Parts                                                                            |
| Ferric chloride      | 2                                                                                |
| Zinc chloride        | 4                                                                                |
| Sodium chloride      | 2                                                                                |
| Ammonium chloride    | 1                                                                                |
| Ferrous chloride     | 2                                                                                |
| Zinc chloride        | 2                                                                                |
| Sodium chloride      | 1                                                                                |
| Ammonium chloride    | 1                                                                                |
| Iron sulphate (ous)  | 2                                                                                |
| Zinc chloride        | 4                                                                                |
| Sodium chloride      | 2                                                                                |
| Ammonium chloride    | 1                                                                                |
| Zinc acetate         | 2                                                                                |
| Zinc chloride        | 4                                                                                |
| Sodium chloride      | 2                                                                                |
| Ammonium chloride    | 1                                                                                |
| Zinc borate          | 2                                                                                |
| Zinc chloride        | 4                                                                                |
| Sodium chloride      | 2                                                                                |
| Ammonium chloride    | 1                                                                                |
| Antimony trichloride | 2                                                                                |
| Zinc chloride        | 4                                                                                |
| Sodium chloride      | 2                                                                                |
| Ammonium chloride    | 1                                                                                |

45 The reasons back of the action which takes place here are obscure and I am therefore leaving open the question as to whether the effect is produced by reason of catalytic action or because of what is popularly known as an affinity of the fluxing material for the metal to be coated and for the lead or because carrying further the "affinity" idea, the fluxing material or catalyst—or whatever it may be—is capable of forming alloy with each of the metals to be coated and the lead, the action being similar to an alloying action but the flux not entering into actual alloy with either to an extent which would deplete it seriously, or whether there be some other reason for the action. At any rate by 50 whatever flux used the lead coating persists through cold-working with amazing tenacity, so much so that I have been required to remove it after complete cold-working, in order that government inspectors can make sure of the surface under the lead.

Another measure of the unusual persistence of the lead coating is the fact that in the rare cases of reannealing, during cold working where my invention has been used, reannealing in a 55 controlled atmosphere (such, for example, as an atmosphere of disassociated anhydrous ammonia) does not disturb the lead coating and continued cold working does not require additional coating.

75 I have had great success in cold working of

metals which have been coated by my invention, which is a tribute to the comparative purity of the lead which I have used, and particularly to the fact that the lead has been substantially free from alloying tin or alloying other metals which would have a hardening effect.

I have found that a better coating of lead is secured where the metal to be coated, herein referred to generally as the "work," is passed through the flux and then is reciprocated or otherwise moved back and forward in the flux and lead. In order that the work may engage different parts of the bath and stir the bath, the work is advanced from one range of reciprocation to another, progressively toward the point of withdrawal from the lead. The work is withdrawn preferably through a clean lead surface since in this way the flux is not given opportunity to form a final coating upon the lead. The reciprocation is not suggested in Figure 1 but the withdrawal through a clean lead surface is.

Mechanism is not necessary for the "reciprocation," as I refer to any movement of the metals to be coated, as any such desired movement of the work articles can be effected by hand manipulation, dipping the articles into the bath in any suitable container, preferably in the form of a cage or basket, closed to retain the work pieces but permitting free flow of bath through it. The basket and work piece content are moved about in the bath as desired. However, an effective movement can be secured by mechanism. For this reason a suitable machine has been illustrated in Figures 3, 4 and 5 and will now be described.

A platform 9 is supported upon legs 10 and 11, resting upon any suitable base, here shown as the upper rim 12 of the pot 52. The platform supports a motor 13 connected by belt 14 with a pulley 15. The speed of rotation is reduced through any suitable gear box 16 so that the rate of rotation of shaft 17 will be low enough for present purposes. The shaft carries a crank arm 18 connected by a pin 19 with a connecting rod 20. The throw of the crank arm may be adjusted by connecting the pin 19 with the crank arm at other points, such as at 21, for example.

A ratchet wheel 22 is mounted upon a shaft 23 supported by bearings upon struts 24. The shaft carries also spaced sprocket wheels 25 upon which operate the chains 26 of a chain conveyor having conveyor bars 27 across from chain to chain constituting flights 28. The bars 27 are merely supports connected with the chain at convenient points by attachment to tabs 29.

A partition or division plate 30 suitably supported from the side structure 31 and brackets 32, dips down into the lead bath 6 to prevent the flux 82 from distributing over the surface of the bath. The flux is otherwise confined by box 33. The conveyor bars on their downward strokes pass through the flux into the bath.

The connecting rod 20 is pivoted to a rocker arm 34 at a distance (rocker arm length or throw) from shaft 23 large enough so that rotation of the crank arm 18 will cause oscillation only of the arm 34. The arm 34 carries a holder 35 for a ratchet plunger 36. The plunger is drawn toward engagement with the teeth of the ratchet wheel by spring 37, capable of being withdrawn therefrom by handle 38 so that the ratchet disc and sprocket wheels can be rotated by hand to any extent desired when the ratchet plunger 36 has been withdrawn from the teeth of the ratchet wheel. This makes it possible to turn 75

the conveyor to any point desired, moving baskets 39 by the flights upon the sprocket chains through the flux back and forth across the flux line.

5 The reciprocation seems to have a scrubbing action and if the metal to be coated be finally taken out of the lead at a lead surface free from flux there seems to be no film of flux on the coating. Even where the metal-coated comes 10 out through flux there is little trace of flux and the flux can be selected to be as little objectionable as possible.

As seen in Figure 4 the preferably closed work cages or baskets for the articles to be coated 15 are hung by hooks 40 from bars or flights 27. The hooks are connected with the bars or flights in a position slightly to the right of that shown in Figure 4, after which the baskets and the hooks are slid to the left so that the hooks 40 20 come beneath guards 41, holding the baskets in position upon the flights, even when the baskets are turned upside down, as takes place when the sprocket chains are moving upwardly to the left (Figure 3) of the partition 30.

25 The lower parts of the sprocket chains pass about wheels 42 down in the bath, which wheels need not be sprocket wheels but may be pulleys merely. Bearings for the pulley shaft 43 are supported by stays 44 extending down from the 30 partition 30. It has not been considered necessary to show the supports in detail, other than to indicate them at 45 in Figure 4.

The pot 52 is conventionally shown as seated in a concrete bed 46 having a rim 47 upon which 35 the flange 48 of the pot may be rested.

In order that the metal of the conveyor, such as the chains and the flights, may not chill the lead bath, a heater is supplied, including a gas pipe 49 controlled by valve 50. It discharges gas 40 through a burner nozzle 51 so that hot air at 52 may be fed through an upright pipe 53 and a manifold 54. The manifold distributes the hot products of combustion against the chain, preferably on the down side of the conveyor, heating the conveyor sufficiently so that there is no chilling of the molten lead. The bath may also be heated separately as by an electrical heating unit within the bath. Heater 55 is conventional and is supplied with current through wires 56 50 protected by conduit 57.

Notwithstanding that there is individual merit in the particular mechanism shown and that this mechanism will be claimed, the drawing is intended to be conventional to the extent that it represents one mechanism by which the baskets for the metal to be coated may be moved back and forward within the lead bath and across the fluid line, and it is the intention to claim the method as well as the mechanism by which this function is secured.

Whether the articles to be coated (work) be moved by hand or by mechanism for the purpose, such, for example, as the one illustrated, the present invention offers considerable advantage in uniformity and completeness of coating to be secured by this movement.

In operation, articles to be coated and subsequently to be cold-processed are placed within the basket and the basket is attached to a flight of the conveyor, after which the ratchet plunger is withdrawn from the teeth of the ratchet wheel while the sprockets and chains are turned to carry the basket through the flux and into the lead bath and back again so that with reciproca-

tion due to the mechanism the basket will reciprocate back and forward past the flux line.

The ratchet tooth is reset within the ratchet wheel at such a point in the revolution of crank arm 18 that the reciprocation will take place initially over the desired range in the depth of the molten pool of lead. The revolution of the crank arm 18 will cause oscillation of the arm 34 with corresponding oscillation of the ratchet wheel and the sprocket wheels, and with successive reversals of limited movements of the sprocket chains.

When there has been sufficient reciprocation of the basket for the articles properly to be coated, the ratchet plunger is withdrawn from the ratchet wheel, the sprocket chains are advanced a distance sufficient to carry the basket through the lead and out to a part of the bath at which reciprocation is within the lead alone and the articles are withdrawn. The ratchet plunger is allowed to enter a different notch in the ratchet wheel. Reciprocation of new basket is begun while other baskets along the conveyor are reciprocated where they may be.

While the movement of the basket has been called reciprocation, because during a considerable part of the distance travelled the container will move in a straight line and back again, as seen in Figure 3, there may also be oscillatory movement of the basket where it travels about the curved portion of the wheel at the bottom of the bath. Adjoining the straight stretches of the sprocket chains there will be movements which will be partially reciprocations and partially oscillations. It is my intention to use "reciprocation" to cover these various movements.

When there has been sufficient reciprocation of the baskets within the molten bath and flux the ratchet tooth is withdrawn from the ratchet wheel and the sprocket chains are turned to bring the baskets out from the bath, the container is drained in a trough 58 or other resting place and is subsequently cooled.

The coating is followed by cold-process working in dies or by other tools securing the lubricant advantages.

The invention has been quite successful in making cartridge casings from a cupped or flat blank which is first cupped and then successively drawn to the final size of the casing needed. With the lead coating I have performed five successive drawing operations before annealing and then, with a controlled atmosphere I have been able to anneal without losing the lead coating, nor the lubricant quality of the lead coating, continuing to perform other successive drawing operations.

The lead coating forms a basis for continuing cold processing without annealing and these operations are contemplated in connection with the coating.

In view of my invention and disclosure variations and modifications to meet individual whims or particular need will doubtless become evident to others skilled in the art, to obtain all or part of the benefits of my invention without copying the structure shown, and I, therefore, claim all such in so far as they fall within the reasonable spirit and scope of my claims.

Having thus described my invention what I claim as new and desire to secure by Letters Patent is:

1. The method of coating a metal cold working blank preparatory to cold working with at least commercially pure lead for lubricating by

the coating during cold working, which comprises forming a bath of at least commercially pure molten lead, floating upon the molten lead a flux comprising a metallic salt which is fusible and relatively stable at a temperature corresponding substantially with that of the molten lead, the salt being selected from the group consisting of acetates, borates, chlorides and sulphates of the metals antimony, bismuth, cadmium and tin, passing the metal cold working blank to be coated repeatedly back and forth across the flux-molten lead interface into the molten lead, and withdrawing the metal cold working blank coated from the molten lead.

2. The method of coating a steel cold working blank preparatory to cold working with at least commercially pure lead for lubricating by the coating during cold working, which comprises forming a bath of at least commercially pure molten lead, floating upon the molten lead a flux comprising a metallic salt which is fusible and relatively stable at a temperature corresponding substantially with that of the molten lead, the salt being selected from the group consisting of acetates, borates, chlorides and sulphates of the metals antimony, bismuth, cadmium and tin, advancing the steel cold working blank through the flux into the molten lead by a back and forth motion which causes an individual point on the blank to move repeatedly across the interface between the flux and the molten lead, and withdrawing the steel cold working blank coated from the molten lead.

3. The method of coating a metal cold working blank preparatory to cold working with at least commercially pure lead for lubricating by the coating during cold working, which comprises forming a bath of at least commercially pure molten lead, floating upon the molten lead a flux comprising a metallic chloride which is fusible and relatively stable at a temperature corresponding substantially with that of the molten lead, the chloride being selected from the group consisting of cadmium chloride and tin chloride, the flux containing at least 10% of cadmium chloride or at least 25% of tin chloride, passing the metal cold working blank to be coated repeatedly back and forth across the flux-molten lead interface into the molten lead, and withdrawing the metal cold working blank coated from the molten lead.

4. The method of coating a metal cold working blank preparatory to cold working with at least commercially pure lead for lubricating by the coating during cold working, which comprises forming a bath of at least commercially pure molten lead, floating upon the molten lead a flux comprising a metallic salt which is fusible and relatively stable at a temperature corresponding substantially with that of the molten lead, the salt being selected from the group consisting of acetates, borates, chlorides and sulphates of the metals antimony, bismuth, cadmium and tin, and at least one chloride of the class consisting of zinc, sodium and ammonium chloride, passing the metal cold working blank to be coated repeatedly back and forth across the flux-molten lead interface into the molten lead, and withdrawing the metal cold working blank coated from the molten lead.

5. The method of coating a metal cold working blank preparatory to cold working with at least commercially pure lead for lubricating by the coating during cold working, which comprises forming a bath of at least commercially pure

molten lead, floating upon the molten lead a flux comprising a metallic salt which is fusible and relatively stable at a temperature corresponding substantially with that of the molten lead, the salt being selected from the group consisting of acetates, borates, chlorides and sulphates of the metals antimony, bismuth, cadmium and tin, and at least two chlorides of the class consisting of zinc, sodium and ammonium chloride, passing the metal cold working blank to be coated repeatedly back and forth across the flux-molten lead interface into the molten lead, and withdrawing the metal cold working blank coated from the molten lead.

6. The method of coating steel with lead for lubrication purposes for cold working, which comprises forming a bath of at least commercially pure molten lead, covering the molten lead bath with a molten flux comprising a sulphate selected from a group consisting of tin sulphate, 15 cadmium sulphate and antimony sulphate, dipping a wrought steel cold working blank repeat-

edly back and forth through and in contact with the flux into the lead bath and withdrawing the steel cold working blank coated with lead from the lead bath at a point where the bath is free 5 from flux.

JACQUES MAGNIN.

REFERENCES CITED

10 The following references are of record in the file of this patent:

UNITED STATES PATENTS

| Number    | Name      | Date          |
|-----------|-----------|---------------|
| 1,189,373 | Maddy     | July 4, 1916  |
| 1,276,978 | Shoemaker | Aug. 28, 1918 |
| 1,548,514 | Dudzeele  | Aug. 4, 1925  |
| 1,572,953 | Pletsch   | Feb. 16, 1926 |
| 2,013,047 | Hand      | Sept. 3, 1935 |
| 2,068,687 | Liban     | Jan. 26, 1937 |
| 2,368,128 | Kinkbone  | Jan. 30, 1945 |
| 2,390,440 | Kalil     | Dec. 4, 1945  |